# EUROPEAN PATENT SPECIFICATION

(11) **EP 3 875 646 B1**
(45) Date of publication and mention of the grant of the patent: **30.07.2025**
(21) Application number: 21158961.9
(22) Date of filing: 24.02.2021
(51) Int. Cl.: D01F 8/04, D01F 8/10, D01F 8/16, D01D 11/06, D02G 3/36, D06M 15/347

(54) **COMPOSITE YARN**
VERBUNDGARN
FIL COMPOSITE

(30) Priority: 03.03.2020 TW 109202337 U
(43) Date of publication of application: 08.09.2021
(73) Proprietor: Lin, Chun Wei, Taichung City (TW)
(72) Inventor: Lin, Chun Wei, Taichung City (TW)
(74) Representative: Melchior, Robin

(56) References cited:
- EP-A1- 1 867 771
- SU-A1- 1 282 222
- US-A- 2 238 694
- US-B1- 10 522 269
- GRASSMANN CARSTEN ET AL: "Recycled Polyvinyl Butyral for Textile Applications", TEXTILE COATING AND LAMINATING CONGRESS, GHENT, 1 September 2019 (2019-09-01), XP055820514, Retrieved from the Internet <URL:https://www.researchgate.net/publication/329363645_Coating_of_Recycled_Polyvinylbutyral_on_Yarns> [retrieved on 20210706]
- GRASSMANN CARSTEN ET AL: "Coating of Recycled Polyvinylbutyral on Yarns", 1 November 2018 (2018-11-01), XP055820517, Retrieved from the Internet <URL:https://www.researchgate.net/publication/329363645_Coating_of_Recycled_Polyvinylbutyral_on_Yarns> [retrieved on 20210702]
- GRASSMANN CARSTEN ET AL: "Investigation of Recycled Polyvinyl Butyral for Yarn Based Textile Coatings", 1 November 2019 (2019-11-01), XP055820506, Retrieved from the Internet <URL:https://www.researchgate.net/publication/337398746_Investigation_of_Recycled_Polyvinyl_Butyral_for_Yarn_Based_Textile_Coatings> [retrieved on 20210702], DOI: 10.13140/RG.2.2.29480.32008
- DATABASE WPI Week 198736, Derwent World Patents Index; AN 1987-255288, XP002803549

## Description

### BACKGROUND

### 1. Field of the Invention

The present disclosure relates to a composite yarn, and more particular to a core-sheath type composite yarn.

### 2. Description of the Prior Art

Conventionally, after a fabric is obtained by weaving with yarns, the whole fabric needs to be subjected to a sizing step or a sticking step at junctions of multiple crossing yarns by a thermoplastic material. After that, the fabric can be subjected to a setting step. However, the above-mentioned process makes the sizing and setting steps more complicated, and characteristics of the resulting fabric will be easily affected. For example, the resulting fabric may be stiff, and the touch of the resulting fabric or the morphology of the resulting fabric may be affected. Further, the thermoplastic material used in the art generally is polyvinyl chloride (PVC), which is toxic and cannot meet the requirements of environmental protection. It can be seen that yarns or the sizing and setting steps after weaving still need to be developed and improved continuously.

### SUMMARY OF THE INVENTION

Compared with PVC, which cannot meet the requirements of environmental protection, polyvinyl butyral (PVB) is a more eco-friendly material. Besides, PVB can be obtained by recycling wasted laminated safety glass; thus, the recycled PVB can meet the requirements of environmental protection and conform to the business model of circular economy. Moreover, the possibility of using the recycled PVB in various textile coating applications has been investigated in several academic researches. For example, Grassmann Carsten et al. have published conference papers such as "Recycled Polyvinyl Butyral for Textile Applications" (presented at the Textile Coating and Laminating Congress in Ghent, September 2019), "Coating of Recycled Polyvinylbutyral on Yarns", and "Investigation of Recycled Polyvinyl Butyral for Yarn Based Textile Coatings". In view of that, if the recycled PVB is applied to a yarn production or the sizing and setting steps after weaving, the defects of the conventional textile manufacturing should be overcome promisingly.

An objective of the instant disclosure is to provide a composite yarn, which is beneficial for setting and reinforcing an obtained fabric comprising the same and meets the requirements of environmental protection.

The present disclosure provides a composite yarn. The composite yarn includes a core and a sheath. The core is made of a thermoplastic material; wherein the thermoplastic material is selected from a group consisting of: a polyester, a polyamide, a polyacrylonitrile and any combination thereof. The sheath, which is formed around the core, is made of a cladding material, and the cladding material comprises PVB and a thermoplastic polyurethane, and the thermoplastic polyurethane (TPU) is in an amount from larger than 0 part by weight to 100 parts by weight relative to 100 parts by weight of the PVB; wherein the PVB has a melt flow rate (MFR) ranging from 2 grams per 10 minutes (g/10 min) to 35 g/10 min. The MFR is measured by a standard method ASTM D1238 at 190°C with 2.16 kilograms (kg) load.

Since the sheath of the composite yarn fully wraps the core, and the sheath is composed of the cladding material comprising PVB, when the composite yarn is subsequently used in manufacture of fabrics, the sheath will help the direct set of the obtained fabrics through a hot-melt step. Thus, a necessary setting step by using a glue or an adhesive film in the conventional process is no longer needed and textile manufacturing will be simplified. In addition, in the cladding material of the instant disclosure, PVB is used to replace PVC, so the composite yarn can meet the requirements of eco-friendliness. Moreover, by controlling the MFR of the PVB of the instant disclosure within a specific range, the PVB will have a suitable flowability during a hot-melt step. Therefore, even though the cladding material does not comprise any plasticizer, the cladding material still can make the surface of the obtained fabric smooth and make the touch of the obtained fabric comfortable.

Preferably, the cladding material may further comprise a polymer material. Specifically, the polymer material may comprise a phenol-formaldehyde resin, an epoxy resin, a poly(methyl methacrylate), an ethylene-vinyl acetate copolymer (EVA), a methyl methacrylate-butadienestyrene copolymer (MBS), a styrene-butadiene block copolymer (SBC) or any combination thereof.

In the present disclosure, the cladding material comprises the TPU, and thus can further adjust the elasticity thereof.

Preferably, the cladding material may further comprise a plasticizer. Specifically, the plasticizer may comprise acetyl tributyl citrate (ATBC), acetyl trioctyl citrate (ATOC), an alkyl benzyl phthalate such as butyl benzyl phthalate, an alkyl phthalate, blown linseed oil, butyl ricinoleate, castor oil, a dialkyl adipate such as dihexyl adipate and dioctyl adipate (DOA), a dialkyl phthalate such as dibutyl phthalate (DBP) and dioctyl phthalate (DOP), di-isononyl-cyclohexane-dicarboxylate (DINCH), ethylene glycol di-N-butyrate, isodecyl diphenyl phosphate, N-ethyl toluenesulfonamide, polyethylene glycol, tert-butylphenyl diphenyl phosphate, toluenesulfonamide, triaryl phosphate ester blend, tributyl citrate (TBC), tricresyl phosphate (TCP), triethyl citrate (TEC), triethylene glycol, triethylene glycol bis(2-ethylhexanoate), triphenyl phosphate (TPP), 2-ethylhexyl diphenyl phosphate or any combination thereof.

In certain embodiments, the plasticizer is in an amount from 20 parts by weight to 100 parts by weight relative to 100 parts by weight of the PVB.

Preferably, the PVB may be obtained by recycling wasted laminated safety glass. In particular, the process of producing the recycled PVB from the wasted laminated safety glass contains a separation procedure and a purification procedure. The separation procedure may comprise steps in sequence: cutting edges of the wasted laminated safety glass that are adhered to impurities, crushing the aforesaid wasted laminated safety glass, soaking the original PVB layer of the aforesaid wasted laminated safety glass, and striking the aforesaid wasted laminated safety glass to make the glass fall off. The purification procedure may comprise steps in sequence: tearing the aforesaid PVB layer, further removing remaining glass, adding magnesium silicate and then drying at 45°C, and finally obtaining the recycled PVB.

Preferably, the PVB has the MFR ranging from 7 g/10 min to 15 g/10 min.

Preferably, the sheath has a thickness ranging from 0.08 millimeters (mm) to 5.0 mm. More preferably, the sheath has the thickness ranging from 0.08 mm to 0.9 mm**.** The thickness of the sheath is a distance defined as a difference between a radius of the composite yarn and a radius of the core.

In accordance with the present disclosure, the core may be a single yarn or a strand. The single yarn with a certain strength and a certain density is produced by two or more staple fibers or filaments which are arranged almost in parallel and then are twisted helically along an axial direction. The strand is composed of two or more single yarns twisted together. Both of the aforesaid single yarn and the aforesaid strand are made of the thermoplastic material.

In accordance with the present disclosure, the composite yarn can be used to produce a fabric by knitting, circular weaving, plain weaving or weaving, but it is not limited thereto.

In accordance with the present disclosure, the fabric produced by the composite yarn can be applied for various purposes such as curtains, carpets, awnings, beach umbrellas, table mats and mobile phone bags, but it is not limited thereto.

Other objectives, advantages and novel features of the disclosure will become more apparent from the following detailed description when taken in conjunction with the accompanying drawings.

### BRIEF DESCRIPTION OF THE DRAWING

Fig. 1 is a structural schematic view showing that a composite yarn of one example in accordance with the instant disclosure.

### DETAILED DESCRIPTION OF THE INVENTION

The following example is not encompassed in the scope of the claims.

With reference to Fig. 1, a composite yarn 1 of Example 1 of the present disclosure comprised a core 10 and a sheath 20.

The core 10 was a single yarn made by twisting multiple polyamide filaments.

The sheath 20 was wrapped around the core 10. The sheath 20 was composed of a cladding material, which comprised PVB and a plasticizer. Provided that the PVB was in an amount of 100 parts by weight, the plasticizer was in an amount of 20 parts by weight.

The PVB had a melt flow rate of 12 g/10 min according to a standard method ASTM D1238 at 190°C with 2.16 kg load.

The PVB was obtained by recycling wasted laminated safety glass.

The sheath 20 had a thickness of 0.25 mm.

In conclusion, the sheath of the composite yarn of the present disclosure is fully wrapped around the core and the sheath is composed of the cladding material comprising PVB, so the sheath can make an obtained fabric set directly through a hot-melt process when the composite yarn is used in subsequent manufacture of fabrics. Therefore, the textile manufacturing will be simplified. In addition, the cladding material is essentially composed of PVB, which can sufficiently meet the requirements of environmental protection, so the composite yarn indeed can achieve the objective of the present disclosure.

## Claims

1. A composite yarn (1), **characterized in that** the composite yarn (1) comprises:
a core (10) which is made of a thermoplastic material; wherein the thermoplastic material is selected from a group consisting of: a polyester, a polyamide, a polyacrylonitrile and any combination thereof; and
a sheath (20) which is formed around the core (10); wherein the sheath (20) is made of a cladding material, and the cladding material comprises polyvinyl butyral and a thermoplastic polyurethane, and the thermoplastic polyurethane is in an amount from larger than 0 part by weight to 100 parts by weight relative to 100 parts by weight of the polyvinyl butyral; wherein the polyvinyl butyral has a melt flow rate ranging from 2 grams per 10 minutes to 35 grams per 10 minutes; the melt flow rate is measured by a standard method ASTM D1238 at 190°C with 2.16 kilograms load.

2. The composite yarn (1) as claimed in claim 1, wherein the sheath (20) has a thickness ranging from 0.08 millimeters to 5.0 millimeters.

3. The composite yarn (1) as claimed in claim 1, wherein the sheath (20) has a thickness ranging from 0.08 millimeters to 0.9 millimeters.

4. The composite yarn (1) as claimed in any one of claims 1 to 3, wherein the cladding material further comprises a plasticizer.

5. The composite yarn (1) as claimed in claim 4, wherein the plasticizer is in an amount from 20 parts by weight to 100 parts by weight relative to 100 parts by weight of the polyvinyl butyral.

6. The composite yarn (1) as claimed in any one of claims 1 to 5, wherein the polyvinyl butyral has the melt flow rate ranging from 7 grams per 10 minutes to 15 grams per 10 minutes; the melt flow rate is measured by the standard method ASTM D1238 at 190°C with 2.16 kilograms load.

## Patentansprüche

1. Verbundgarn (1),
**dadurch gekennzeichnet**
**dass** das Verbundgarn (1)
- einen Kern (10), der aus einem thermoplastischen Material hergestellt ist, wobei das thermoplastische Material aus einer Gruppe ausgewählt ist, bestehend aus: einem Polyester, einem Polyamid, einem Polyacrylnitril und Kombinationen davon; und
- eine Ummantelung (20), die um den Kern (10) gebildet ist; wobei die Ummantelung (20) aus einem Ummantelungsmaterial hergestellt ist und das Ummantelungsmaterial Polyvinylbutyral und ein thermoplastisches Polyurethan umfasst,
umfasst und das thermoplastische Polyurethan in einer Menge von mehr als 0 bis 100 Gewichtsteilen, bezogen auf 100 Gewichtsteile des Polyvinylbutyrals liegt; wobei das Polyvinylbutyral einen Schmelzfließindex im Bereich von 2 bis 35 Gramm pro 10 Minuten aufweist und der Schmelzfließindex nach einer Standardmethode ASTM D1238 bei 190°C mit 2,16 Kilogramm Last gemessen wurde.

2. Verbundgarn (1), nach Anspruch 1,
wobei die Ummantelung (20) eine Dicke im Bereich von 0,08 bis 5,0 Millimetern aufweist.

3. Verbundgarn (1), nach Anspruch 1,
wobei die Ummantelung (20) eine Dicke im Bereich von 0,08 bis 0,9 Millimetern aufweist.

4. Verbundgarn (1), nach einem der Ansprüche 1 bis 3,
wobei das Ummantelungsmaterial ferner einen Weichmacher enthält.

5. Verbundgarn (1) nach Anspruch 4,
wobei der Weichmacher in einer Menge von 20 bis 100 Gewichtsteilen, bezogen auf 100 Gewichtsteile des Polyvinylbutyrals, vorliegt.

6. Das Verbundgarn (1) nach einem der Ansprüche 1 bis 5,
wobei das Polyvinylbutyral einen Schmelzfließindex im Bereich von 7 bis 15 Gramm pro 10 Minuten aufweist und der Schmelzfließindex nach der Standardmethode ASTM D1238 bei 190°C mit 2,16 Kilogramm Last gemessen wurde.

## Revendications

1. - Fil composite (1), **caractérisé par le fait que** le fil composite (1) comprend :
- une âme (10) qui est faite d'un matériau thermoplastique, le matériau thermoplastique étant choisi dans un groupe consistant en : un polyester, un polyamide, un polyacrylonitrile et toute combinaison de ceux-ci ; et
- une gaine (20) qui est formée autour de l'âme (10), la gaine (20) étant faite d'un matériau de revêtement, et le matériau de revêtement comprenant du poly(butyral vinylique) et un polyuréthane thermoplastique, et le polyuréthane thermoplastique est dans une quantité de plus de 0 partie en poids à 100 parties en poids par rapport à 100 parties en poids du poly(butyral vinylique), le poly(butyral vinylique) ayant un indice de fluidité à chaud se situant dans la plage de 2 grammes par 10 minutes à 35 grammes par 10 minutes, l'indice de fluidité à chaud étant mesuré par une méthode standard ASTM D1238 à 190°C avec une charge de 2,16 kilogrammes.

2. - Fil composite (1) selon la revendication 1, dans lequel la gaine (20) a une épaisseur se situant dans la plage de 0,08 millimètre à 5,0 millimètres.

3. - Fil composite (1) selon la revendication 1, dans lequel la gaine (20) a une épaisseur se situant dans la plage de 0,08 millimètre à 0,9 millimètre.

4. - Fil composite (1) selon l'une quelconque des revendications 1 à **3,** dans lequel le matériau de revêtement comprend en outre un plastifiant.

5. - Fil composite (1) selon la revendication 4, dans lequel le plastifiant est dans une quantité de 20 parties en poids à 100 parties en poids par rapport à 100 parties en poids du poly(butyral vinylique).

6. - Fil composite (1) selon l'une quelconque des revendications 1 à 5, dans lequel le poly(butyral vinylique) a l'indice de fluidité à chaud se situant dans la plage de 7 grammes par 10 minutes à 15 grammes par 10 minutes, l'indice de fluidité à chaud étant mesuré par la méthode standard ASTM D1238 à 190°C avec une charge de 2,16 kilogrammes.
